

## [54] WASHING POLYMERS

[76] Inventors: **Harold S. Akrongold; Rochelle Akrongold**, both of 39 Cathay Rd., East Rockaway, N.Y.

[\*] Notice: The portion of the term of this patent subsequent to Apr. 4, 1989, has been disclaimed.

[22] Filed: Apr. 2, 1973

[21] Appl. No.: 347,396

[52] U.S. Cl. .... 252/91; 252/106; 252/117; 252/544; 252/546

[51] Int. Cl. .... C11d 17/04

[58] Field of Search .... 252/91, 117, 106, 544, 252/546, DIG. 2

## [56] References Cited

## UNITED STATES PATENTS

2,450,940 10/1948 Cowan et al. .... 260/404.5

|           |         |                       |           |
|-----------|---------|-----------------------|-----------|
| 3,148,125 | 9/1964  | Strianse et al. ....  | 424/64    |
| 3,157,681 | 11/1964 | Fischer ....          | 260/407   |
| 3,256,304 | 6/1966  | Fischer et al. ....   | 260/407   |
| 3,383,320 | 5/1968  | Bell....              | 252/132   |
| 3,575,883 | 4/1971  | Foley ....            | 252/546 X |
| 3,654,167 | 4/1972  | Akrongold et al. .... | 252/544 X |
| 3,663,694 | 5/1972  | Hall ....             | 252/106 X |
| 3,671,630 | 6/1972  | Carroll et al. ....   | 252/106 X |

Primary Examiner—Benjamin R. Padgett

Assistant Examiner—E. A. Miller

Attorney, Agent, or Firm—Arthur A. Jacobs, Esq.

## [57]

## ABSTRACT

A hydrophilic gel of a polymeric fat acid polyamide, and a diethanolamide of a fatty acid or a branched chain fatty acid.

14 Claims, No Drawings

1  
WASHING POLYMERS

This invention relates to polymerized fatty acid polyamides and diethanolamide of fatty acids which can be used as detergent and detergent soap type washing polymers.

More particularly, this invention relates to washing polymers in the form of gels derived from polyamide resins which may be either transparent, translucent or opaque and which have many properties that make them unique.

As used herein, the term "gel" is meant to include hydrophilic compositions which range from solids to liquids of the type encountered in the liquid household detergents. However, the viscosity of the composition of this invention is readily controlled during processing depending upon the use desired for the composition.

When practicing a preferred embodiment of this invention, a washing polymer is obtained by mixing, while heating, 0.5-95 parts by weight of a polymeric fat acid polyamide, preferably polymerized tall oil fat acid polyamide, and 1-95, preferably 10-80, and most preferably 25-60, parts by weight of a fatty acid compound such as diethanolamide of a fatty acid or a branched chain fatty acid neutralized with di- or tri-ethanolamine or mixtures thereof. The diethanolamide of the fatty acid or the branched chain fatty acid contains 6-22 carbon atoms, preferably 8-12 carbon atoms. The polymeric fat acid polyamide and either the diethanolamide or the branched chain fatty acid are heated to the melting point of the polyamide and then held for a period of time, up to 4 hours, preferably 15-30 minutes, at the melting point of the polyamide. The heated mixture is allowed to cool and form a gel which can be used as a washing polymer.

The subject matter of the present invention is substantially disclosed in applicants' U.S. Pat. No. 3,654,167, dated Apr. 4, 1972, which patent is incorporated by reference herein.

In the aforesaid U.S. Pat. No. 3,654,167, the disclosure and claims indicated that it was necessary to use 5-95 parts by weight of a polymeric fat acid polyamide. It has now been found that the desired results are also satisfactorily obtained when the proportion of the polymeric fat acid polyamide is as low as 0.5 parts by weight.

The following examples illustrate other compositions embodying the present invention in addition to those disclosed in the aforesaid U.S. Pat. No. 3,654,167:

EXAMPLE 1

| Components                                                                                              | Parts by Weight |
|---------------------------------------------------------------------------------------------------------|-----------------|
| "Emerez 1530" (polymerized fatty acid polyamide)                                                        | 12              |
| "Shercomid CDO Extra" (diethanolamide of mixed fatty acids)                                             | 18              |
| "Standopol 7021 Concentrate" (Henkel Chemical Co. — mixture of di- and tri-ethanolamine lauryl sulfate) | 70              |

The "Emerez 1530" and the "Shercomid CDO Extra" are mixed together under agitation at a temperature of between the melting point (about 115°-120°C) of the polyamide and about 20°C above said melting point for about 20 minutes. While maintaining this temperature, the "Standopol 7021 Concentrate" is added

under agitation, after which the temperature is lowered to room temperature.

2  
EXAMPLE 2

| Components                                         | Parts by Weight |
|----------------------------------------------------|-----------------|
| "Versalon 1200" (polymerized fatty acid polyamide) | 3.5             |
| "Shercomid CDO Extra"                              | 12.5            |
| "Standopol 7021 Concentrate"                       | 84.0            |

The same procedure is used as in Example 1 except for the substitution of the "Versalon 1200" for the "Emerez 1530."

EXAMPLE 3

| Components                                                                                                           | Parts by Weight |
|----------------------------------------------------------------------------------------------------------------------|-----------------|
| "Versalon 1200"                                                                                                      | 0.5             |
| "Shercomid CDO Extra"                                                                                                | 10.5            |
| "Standopol 7021 Concentrate"                                                                                         | 87.0            |
| Polyethylene granules (mixture of granules of size ranging between about 0.0001 inch to about 1/32 inch in diameter) | 2.0             |

The same procedure is used as in Examples 1 and 2 except that the temperature of the mixture of the first three components is first brought down to about 70°C, at which temperature the polyethylene granules are added with agitation. The mixture is then cooled to room temperature. The resultant product, wherein the polyethylene granules are suspended in the gel, may be most satisfactorily used as an acne scrub.

EXAMPLE 4

| Components                   | Parts by Weight |
|------------------------------|-----------------|
| "Versalon 1200"              | 0.5             |
| "Standopol 7021 Concentrate" | 90.0            |

The same procedure is used as in Example 1 except that the "Versalon 1200" is substituted for the "Emerez 1530". The resultant product is a "flowable gel"; that is, although it does not pour like water, if the fingers are inserted therein it feels like a liquid. It has the consistency of a "Carbopol" type or free-flowing, 50 gel. It is highly satisfactory for use as a facial scrub cleaner.

EXAMPLE 5

| Components                   | Parts by Weight |
|------------------------------|-----------------|
| "Versalon 1200"              | 4.0             |
| Isostearic acid              | 10.0            |
| Diethanolamine (99%)         | 10.0            |
| "Standopol 7021 Concentrate" | 76.0            |

The first three components are heated to at least the melting point of the "Versalon 1200", preferably about 160°C. It is held at that temperature for about 1 hour. The "Standopol 7021 Concentrate" is then added with agitation. The mixture is then cooled with agitation to about 65°C, at which time it is poured into a mold or tube where it is permitted to cool to room temperature.

The resultant product is a shaving cream which has a high degree of protective action against nicks and cuts on the skin by providing a very thin film on the skin. It provides a gliding action similar to nylon ball bearings.

#### EXAMPLE 6

| Components                                        | Parts by Weight |
|---------------------------------------------------|-----------------|
| "Versalon 1200"                                   | 4.0             |
| "Shercomid CDO Extra"                             | 16.0            |
| "Kaydol" mineral oil<br>(Sonnenborn Chemical Co.) | 5.0             |
| Isopropyl myristate                               | 2.0             |
| Oleyl alcohol                                     | 2.0             |
| "Standopol 7021 Concentrate"                      | 71.0            |

The same general procedure is used as in Example 1, with the mineral oil, the isopropyl myristate and the alcohol being added together with the "Standopol 7021 Concentrate." The resultant product is a highly satisfactory bath oil-washing gel.

#### EXAMPLE 7

| Components                                                        | Parts by Weight |
|-------------------------------------------------------------------|-----------------|
| "Emerez 1530"                                                     | 2.0             |
| "Shercomid CDO Extra"                                             | 10.0            |
| "Fractar-5" (a tar fraction sold<br>by the Texas Pharmacol Corp.) | 5.0             |
| "Standopol 7021 Concentrate"                                      | 83.0            |

The same procedure is used as in Example 3, the tar fraction being added in place of the polyethylene granules. This product is a tar gel which is also useful in the treatment of acne.

In general, the gels of this invention are useful, in addition to their other functions, as lubricants between the skin or other tissue and other substances which may otherwise have some abrasive effect. Furthermore, they can also be effectively used as lubricating means for mechanical moving parts such as gears, bearings, automobile assemblies, etc. In essence, therefore, they are highly effective general lubricants.

A particular product embodying this invention is a facial washing bar that is unusually soft to the face and other skin areas. This product comprises a polyurethane sponge bar combined with a composition of the type illustrated by the above examples. The following example exemplifies such product:

#### EXAMPLE 8

A hollow box-like container made of rigid plastic, such as polyethylene or the like, and provided with an open top face, is filled with the gel composition of Example 1. A sponge-like pad of foam construction, having a size and contour to closely fit within the open face of the box-like container, is pushed through the open face of the container, the pad being of a size to extend outwardly of the open face. The gel composition impregnates the foam pad up to a position just below the rim defining the open face of the container. The resulting product has the general appearance of a hair brush with the container forming the solid backing or handle while the outwardly-extending portion of the foam pad takes the place of the brush.

Although any foam-type pad may be used, the preferable material is a polyurethane foam, and the most

preferable material is the so-called "Nerf" foam (a polyether-polyurethane foam modified by the addition of a fire-retardant material — sold by the Okenel Corporation, Lyndhurst, New Jersey and by the Crest Foam Corporation, Moonachie, New Jersey). This particular material, which is unusually soft, is not reticulated as most other foams but is, nevertheless, impregnated by the gel composition, possibly by capillary action, although the exact mechanism of the action is not actually known.

The product made in the above manner can be used on very delicate tissue, such as acne tissue, which would be broken by other rougher foams.

This invention also includes within its scope, an aerosol shave cream which has a nylon ball-bearing type action on the skin and which may also be used as a body lotion to decrease friction between body tissue and synthetic fiber garments, such as nylon, "Acrilan," acetate, polyesters, etc., which often produce chafing on sensitive skin. This composition, although also acting as a lubricant, is somewhat different from those disclosed above in that it is prepared by forming two separate phases and then combining them. This is illustrated by the following example:

#### EXAMPLE 9

| Phase "A"                                                        | Components | Parts by Weight |
|------------------------------------------------------------------|------------|-----------------|
| Coconut fatty acid ("Weccaline 1260A" sold by Drew Chemical Co.) | 1.5        |                 |
| Stearic acid (triple-pressed)                                    | 7.5        |                 |
| "Kaydol" mineral oil 345/355                                     | 1.0        |                 |
| "Ceresynt D" (proprietary formulation of VanDyke Chemical Co.)   | 2.0        |                 |
| "Versalon 1140"                                                  | 3.5        |                 |
| "Shercomid CDO Extra"                                            | 3.5        |                 |

  

| Phase "B"                                                            | Components | Parts by Weight |
|----------------------------------------------------------------------|------------|-----------------|
| "Ceraphyl 60" (quaternized gluconamide sold by VanDyke Chemical Co.) | 1.5        |                 |
| Potassium hydroxide pellets                                          | 0.75       |                 |
| Sodium hydroxide pellets                                             | 0.35       |                 |
| Triethanolamine                                                      | 1.10       |                 |
| Sorbitol (70% aqueous solution)                                      | 5.00       |                 |
| Water                                                                | 72.30      |                 |

The "Versalon 1140" and the "Shercomid CDO Extra" are first pre-heated to about 160°C for about 15 minutes. The remaining components of Phase "A" are then added with agitation, after which the mixture is cooled to about 75°-80°C. The components of Phase "B" are separately mixed and heated to about 75°-80°C. Phase "B" is then added to Phase "A" with agitation and the mixture is then held at about 75°-80°C for about 15 minutes in order to obtain saponification. The mixture is then cooled, with continuous agitation, to about 30°C. The mixture is then pressure filled into a six-ounce aerosol can together with "Freon 12" (DuPont) as a propellant in the proportion of 91.0 parts by weight of the mixture and 9.0 parts by weight of the propellant.

The invention claimed is:

1. A detergent composition consisting essentially of a hydrophilic gel reaction product formed by mixing:
  - I. 0.5-95 parts by weight of a polyamide resin product having a molecular weight of about 2,000 to about 10,000 and formed by the reaction of:

- a. a polymerized 16 to 24 carbon atom fatty acid; and
  - b. a diamine selected from the group consisting of alkylene diamines having 2-6 carbon atoms in the alkylene group, bis (aminoethyl) benzene, cyclohexyl bis (methylamine), dimeric fat diamine, and mixtures thereof; and
- II. 1-95 parts by weight of either
- a. a diethanolamide of a fatty acid having 6-22 carbon atoms or
  - b. a branched chain fatty acid having 6-22 carbon atoms, the total mixture, when containing said branched chain fatty acid, being neutralized with either diethanolamine, triethanolamine, or mixtures thereof.
2. A composition as in claim 1 wherein the diethanolamide of a fatty acid is the reaction product of 2 moles of diethanolamine and 1 mole of a fatty acid.
3. A composition as in claim 1 wherein the diethanolamide or the branched chain fatty acid is present in an amount of 10-80 parts by weight.
4. A composition as in claim 1 wherein the diethanolamide or the branched chain fatty acid is present in an amount of 25-60 parts by weight.
5. A composition as in claim 1 wherein the diamine is an alkylene diamine having 2-6 carbon atoms in the

alkylene group.

6. A composition as in claim 1 wherein the diethanolamide or the branched chain fatty acid has 8-12 carbon atoms.

7. A composition as in claim 1 including up to 50% by weight of the composition of n-propyl alcohol.

8. The composition of claim 1 and including from about 5 to 75% by weight of a surfactant selected from the group consisting of anionic, cationic, nonionic and

10 amphoteric surfactants.

9. The composition of claim 1 and including soap in an amount up to 95% by weight of the composition.

10. The composition of claim 1, said composition being transparent.

15 11. The composition of claim 1 wherein said composition is a body having an abrasive body embedded therein.

12. The composition of claim 11 wherein said abrasive body is a member of the group consisting of sponge, plastic wool, steel wool, tar and polyethylene granules.

13. The composition of claim 1 and including an effective amount of perfume.

14. The composition of claim 1 and including an effective amount of a dye.

\* \* \* \* \*